

Aug. 14, 1934.

E. A. JONES

1,969,886

METHOD OF MANUFACTURING FERRO ALLOYS

Filed May 23, 1932



INVENTOR.  
Edwin A. Jones,  
BY *Honey Cole*.  
ATTORNEYS.

## UNITED STATES PATENT OFFICE

1,969,886

METHOD OF MANUFACTURING FERRO  
ALLOYS

Edwin A. Jones, Jackson, Ohio

Application May 23, 1932, Serial No. 613,099

5 Claims. (Cl. 75—17)

My invention relates to the manufacture of alloys, such for instance as those designed to be remelted and used in the manufacture of cast iron, steel, or special alloy castings; particularly 5 ferro alloys having a high silicon content.

One of the principal objects of my invention is to provide a method of manufacturing alloys which is of great advantage from the standpoint of economy of time and expense required 10 in the electric furnace operation for the refining of the alloy and bringing it to the desired characteristics.

Another object is to provide a method of manufacturing alloys which is characterized by more 15 economical use of alloy additions, due to the comparatively short heating and refining period for conditioning the metal; equally good results being obtained by my method with the use of smaller additions of costly alloying materials as with other methods requiring longer 20 periods of time and the additions of greater amounts of alloying materials.

A further object of my invention is to provide a method of manufacturing alloys which 25 has the advantage of affording better conditions than in the usual methods for eliminating possible harmful effects from the formation of oxides or the absorption of carbon. For instance, the metal may be obtained from the blast furnace at relatively low temperatures, thus preventing 30 harmful foreign elements from being absorbed by the iron that would, if the smelting were done at higher temperatures, go over into the finished alloy and contaminate the same, and the purer metal thus obtained from the blast 35 furnace at relatively low temperatures can be brought in the electric furnace to the required composition by making the desired alloying additions.

Another object is to provide a method which 40 allows the electrodes to be lowered to the proper extent into the charge at the beginning of the operation in the electric furnace, to thereby lower the smelting zone and prevent the current from shunting into the top of the charge and 45 thus result in less effective smelting.

While I have chosen as an illustration an apparatus and method for the manufacture of iron alloys high in silicious content, it will be understood that this is done for purposes of illustration only, and it is not intended that the invention as hereinafter more particularly described and claimed shall be confined, except as restricted by the prior art, to the particular 50 method and apparatus described.

The present commercial methods used in the manufacture of ferro alloys in the electric furnace have many difficult problems. Usually metallic scrap, such as borings, turnings, sheet bundles, etc., is charged into the electric furnace 55

with the proper proportions of manganese ores, silicon in the form of silica sand or ground quartz (SiO<sub>2</sub>), chrome, nickel, titanium, etc., (depending upon what alloy or combination of alloys with iron is desired). Carbon, usually in the 65 form of coke breeze, is introduced throughout the melt to facilitate the passing of the current through the melt, particularly at the beginning of a heat when the furnace burden is cold. It requires several minutes after the current has 70 been turned on for the metal to become molten, after which the electrodes may be lowered into the bath, to thereby come into better contact and effect a more even and economical operation. The current is allowed to pass into the melt to 75 bring the charge to the desired character, after which the content of the furnace is poured into molds or blocks, and when cool is ready for shipment.

But this method, as stated, has objectionable 80 features which my invention is designed to overcome. One of the several difficulties with the commercial methods is the high cost of the melting down period or the initial melt period which brings the charge into a molten condition, for 85 during the melting down period, notwithstanding the carbon addition, the electric load is irregular and is at its peak due to uneven contact with the burden, and to contact with cold scrap. In addition to the high cost of power, the 90 irregular and peak load is injurious both to the carbon electrodes and to the refractory linings of the electric furnace.

According to my method this costly "melting down period", or initial stage in the electric furnace, is greatly reduced or totally eliminated, depending upon the particular alloy being made, the period in every case being partially eliminated. In addition to this saving, my process as a 95 whole is speeded, and the conditions thus prevailing favor the elimination of harmful effects upon the alloy which may result from the present methods, such as the forming of harmful oxides or the picking up of carbon.

In the drawing, which is a diagrammatic vertical sectional view, I have illustrated an installation suitable for the carrying out of my process.

In the drawing, 1 represents a blast furnace, equipped with a tapping notch 2, the furnace being supplied with tuyères 3. A receiving ladle is 110 illustrated at 4, a gas furnace at 5, equipped with a gas burner 6 and a gas head connecting the blast furnace with the gas furnace is indicated at 6'. The contents of the gas furnace may be tapped off at 7 into the ladle 4.

An electric furnace is indicated at 10 and it may be mounted for tilting as at 11. The electrodes are indicated at 12, and the holders at 13. Apparatus for handling the electrode and actuat- 115

ing the furnace is indicated generally at 14. Molds into which the electric furnace contents may be poured are indicated at 15. An overhead crane is indicated at 16.

5 Briefly stated, according to one method I may follow, the ore, etc., is charged into the blast furnace and smelted, resulting in the manufacture of a silicon iron ranging from 6% to 16% in silicon content. This special high silicon iron is 10 tapped from the furnace into a ladle, and is transferred by means of the crane and introduced into the electric furnace. To this molten metal any one or more raw additions are made in the form of chrome ore, manganese ore, quartz, nickel, etc. 15 Also scrap additions may be made, such as borings and turnings, to give necessary iron additions. The raw additions may be added to the molten metal in the electric furnace in a cold state, or they may have been put through a preliminary heating in the gas furnace 5, which furnace is supplied by gas through the header 6 from that taken off of the blast furnace operation. After melting in the gas furnace, (if this intermediate step has been used) the additions may 20 be tapped off into the receiving ladle 4, and transferred by the crane to the electric furnace to be added to the melt therein. Whether the intermediate heating step has been used or not, when 25 the electric furnace has been charged the current is then passed through the melt in the electric furnace until the molten mass has become thoroughly mixed and the proper composition of mixture is reached. The metal is then poured 30 from the electric furnace into sand molds, chill molds, or a pigging machine, and cast into convenient size for handling. The product thus obtained is then an alloy such as ferro-chrome, silico-spiegel, ferro-silicon, etc., and is shipped as 35 40 such to users making all kinds of castings through the ordinary processes of steel or cast iron making.

I may, in those instances where it is found desirable, transfer the iron from the blast furnace to the gas furnace, and there make the additions of other materials desired for the particular alloy being made. These materials may be in a pre-heated condition in the gas furnace at the time of the introduction of the silicon iron, 45 or may be introduced into the gas furnace in a cold state. After the treating in the gas furnace the melt may be transferred to the electric furnace and there refined; whatever small additions, if any are needed to bring the alloy to the desired composition, being made during the refining period in the electric furnace.

50 As a specific example of making an alloy (in this case a 50% ferro-silicon) by my process, I note the following:

(a) *Making 10% Si. pig in the blast furnace*

The following charge of iron ore, lime stone, and fuel is fed into the top of the blast furnace 55 1,—

|           |       |                      |
|-----------|-------|----------------------|
| Tilden    | 4200# | Pig iron 10% silicon |
| Bennett   | 2000# |                      |
| Morris    | 3000# |                      |
| Gardner   | 1200# |                      |
| Limestone | 2800# |                      |

75 The compositions of the iron ores referred to

above may, by way of an illustrative example, be as follows:

|         | Iron  | Phosphorus | Silica | Manganese | Aluminum | Lime | Magnesium | Loss by ignition | 80 |
|---------|-------|------------|--------|-----------|----------|------|-----------|------------------|----|
| Tilden  | 40.35 | .050       | 40.30  | .07       | .96      | .35  | .29       | .40              |    |
| Bennett | 56.30 | .076       | 8.80   | 1.25      | 2.10     | .20  | .17       | 6.20             |    |
| Morris  | 59.15 | .066       | 8.30   | .44       | 2.47     | 1.06 | .29       | 2.83             |    |
| Gardner | 51.00 | .036       | 3.42   | .24       | 1.41     | 2.50 | 1.14      |                  | 85 |

(Above Dried 212° F.)

As the charge passes down through the furnace, it is pre-heated by the combustion of carbon-monoxide rising from the tuyère zone below. As 90 the charge passes through the tuyère zone, the reduction of the alloy of iron and silicon takes place. The iron and silicon passes on down into the final zone, or hearth zone, and is tapped off. The wash or slag lies directly above the iron and 95 is tapped off prior to tapping the furnace for metal.

(b) *Introduction into the gas furnace*

The high-silicon iron (pig iron 10% silicon) is 100 then transferred by ladle into the gas furnace 5 in which have been placed other materials to bring the alloy to the desired composition (in this example 50% ferro-silicon). The charge placed in the gas furnace may be as follows,—

4480# 10% silicon pig

+  
1690# Millscale (often referred to as "mill cinder" and which contains a high percentage of a solid solution of ferrous silicate and 110 iron oxide)

8690# Silica rock

2600# Coke

The gas furnace is operated over a sufficient period of time to bring the entire charge to a pre-heated or a molten state before its introduction into the electric furnace for its final refining. During the treatment in the gas furnace, the following re-action is initiated,—



(c) *Treatment in the electric furnace*

The molten mixture tapped off from the gas furnace is then transferred to the electric furnace. Here the refining period takes place and the reaction is completed. Small additions, if needed, may be used to bring the alloy to the desired composition. After sufficient heat has been passed through the charge in the electric furnace 125 to refine the alloy and bring it to the desired characteristics, the electrodes are raised and the furnace is tilted and the alloy poured in the molds 130 for cooling. The final product obtained in the electric furnace will be,—

13000#—50% Ferro-Silicon

It will be understood that my process is not limited to this alloy, but may be used for the manufacture of a number of ferro-alloys by the 140 introduction into the gas or electric furnace, or both, of materials differing, in part, from those used in the foregoing example.

The electric furnace may be of any standard type. It may be of the tilting or stationary type. The most economical type of furnace for this method of alloying is the arc type where the electrodes, by a lowering and raising device, can be allowed to submerge into the bath to thereby 145

lower the smelting zone, and to allow the current to come into better contact with the alloy.

In the case where introduction of the silicon iron into the electric furnace in the molten state directly from the blast furnace takes place, the iron may be mixed with metals or alloys, one or both, in the cold state, or after having been first pre-heated in the gas furnace. In either case, the introduction of the molten silicon iron tends to melt the additions so as to make the electric furnace operation a short and steady process, without undue wear on the electrodes or the lining materials of the furnace.

My method requires only from fifteen to forty-five minutes treatment of the melt in the electric furnace, the time depending upon the kind of alloy being manufactured, some requiring a longer period to be properly mixed and brought to the required characteristics. This electric furnace operation period required in my method is of much shorter duration however than that of any existing methods for the production of alloys known to me.

It will be observed from the foregoing that my process has the advantage of greater economy in the manufacture of alloys from the standpoint of time required in the electric furnace operation, which operation is very costly. Further, my invention has the advantage of more economical use in alloy additions, due to the shorter heating and refining period, with as good results being obtained by the use of smaller additions of costly alloying materials as with other methods in which greater additions of alloying materials are required. Also, my method has the advantage of better conditions for eliminating possible harmful materials which the alloy may absorb from being held over longer periods of time at high temperatures. Due to the molten condition of the charge when it comes in contact with the electric furnace, my method has the advantage of permitting the electrode to be lowered to the proper degree into the charge with ease, thereby lowering the smelting zone and preventing the electric current from shunting into the top of the charge and causing less effective smelting. Furthermore, where the intermediate step of treating the melt from the blast furnace in the gas furnace, or of pre-heating the additions in the gas furnace, is used, great economy results from the use of the products of combustion generated in the blast furnace, thus effecting material savings to render the process extremely economical in commercial operation.

Having thus described my invention what I claim as new and desire to secure by U. S. Letters Patent is:—

1. The method of manufacturing a high silicon

alloy comprising smelting a charge suitable for the production of a high silicon pig iron in a blast furnace, transferring the high silicon iron from the blast furnace into a gas furnace and there introducing into the high silicon iron materials for bringing the alloy to the desired composition, heating the charge in the gas furnace until it has obtained the proper fluidity, transferring the charge from the gas furnace to an electric furnace and therein refining the charge and making such small additions of materials as are required to bring the alloy to the desired characteristics while regulating the temperature of the charge.

2. The method of manufacturing ferro alloys which comprises smelting a charge of silicious iron ore, lime stone, and fuel in a blast furnace, tapping off the high silicon ferro alloy resulting from the smelting of the charge, and transferring it to an electric furnace, adding to the charge in the electric furnace additional silicious alloying materials required to bring the finished alloy to the desired composition, and heating the mixture in the electric furnace until it is completely alloyed.

3. The method of manufacturing ferro alloys such for instance as those used in steel making and special alloyed cast steel or cast iron which comprises smelting a silicious charge in a blast furnace, tapping off the alloy resulting from the smelting of the charge, transferring it to an electric furnace and therein making such additions of silicious and other materials as are required to bring the finished alloy to the desired composition while regulating the temperature of the charge.

4. The method of manufacturing ferro alloys which comprises smelting a charge of silicious iron ore, limestone, and fuel in a blast furnace, tapping off the silicon ferro alloy resulting from the smelting of the charge and transferring it to an electric furnace, adding to the charge in the electric furnace a silicious compound and a reducing agent in quantities sufficient to introduce upon the reaction of the materials added, sufficient silicon into the alloy to raise it to the desired final content, and heating the mixture in the electric furnace until completely alloyed.

5. The method of producing ferro alloys as end products which comprises producing a ferro alloy having a high silicon content in a blast furnace, transferring such alloy while molten to an electric furnace, adding to the charge in the electric furnace such additions as are required to raise the silicon content to the desired percentage in the finished alloy, and heating the mixture in the electric furnace until it is completely alloyed.

EDWIN A. JONES.